

[54] PROCESS FOR PRODUCING A BULKY YARN

[75] Inventors: **Fumishige Maruyama; Toshiyuki Yasui; Kaoru Asada**, all of Komatsu, Japan

[73] Assignees: **Teijin Limited, Osaka; Teijin Modern Yarn Co., Ltd.**, Komatsu-shi, Ishikawa-ken, both of Japan

[22] Filed: **Dec. 17, 1971**

[21] Appl. No.: **209,115**

[30] Foreign Application Priority Data

Dec. 19, 1970 Japan ..... 45-114882

[52] U.S. Cl. ..... 57/157 TS, 57/34 HS

[51] Int. Cl. ..... D02j 1/20

[58] Field of Search 57/34 R, 34 B, 34 HS, 157 TS, 57/157 R, 157 MS, 157 F

[56]

References Cited

UNITED STATES PATENTS

|           |         |                   |             |
|-----------|---------|-------------------|-------------|
| 3,041,814 | 7/1962  | Held .....        | 57/157 TS X |
| 3,137,119 | 6/1964  | Crouzet .....     | 57/157 TS X |
| 3,309,855 | 3/1967  | Stoll et al. .... | 57/157 F X  |
| 3,543,505 | 12/1970 | Stutz .....       | 57/157 TS   |

Primary Examiner—Donald E. Watkins  
Attorney, Agent, or Firm—Sherman & Shalloway

[57]

ABSTRACT

A method of producing a bulky yarn having a controlled residual torque, which comprises subjecting a thermoplastic synthetic filament yarn to a series of twisting, heat-setting on a first heater, and untwisting, feeding the yarn into a second heater while rotating it by means of a fluid nozzle and re-heat-setting the yarn in the second heater, the yarn being maintained in a substantially relaxed state during the rotation by the fluid nozzle and the re-heat-setting by the second heater.

20 Claims, 11 Drawing Figures



PATENTED JUL 30 1974

3,826,075

**FIG. 1**



**FIG. 2**



**FIG. 3**



**FIG. 4**



**FIG. 5**



**FIG. 6**



**FIG. 7**



**FIG. 8**



**FIG. 9**



**FIG. 10**

**FIG. 11**

## PROCESS FOR PRODUCING A BULKY YARN

This invention relates to a process for producing a yarn having high bulk and controlled residual torque. More specifically, the invention relates to a process for producing a bulky yarn having controlled residual torque by subjecting a thermoplastic synthetic filament yarn to a continuous series of twisting, heat-setting, and untwisting steps, and then again heat-treating it in a substantially relaxed condition.

A number of methods have been proposed previously for the production of bulky yarns. These methods, for example, include a method comprising three steps of heating, heatsetting, and untwisting (German Pat. No. 618,050 and Japanese Pat. No. 130,429), the so-called false-twisting method in which heating, heat-setting, and untwisting are performed in one step (British Pat. No. 424,880), a modified false twist method wherein bulky yarns obtained by false-twisting are simultaneously heat-set, and a method wherein the bulky yarns obtained by false-twisting are again heat-set by heating.

The bulky yarns produced by these methods have different forms of crimp or yarn quality such as crimpability. These conventional methods, however, cannot at all exert a free control of the residual torque while retaining the desirable bulkiness.

Yarns produced by a series of twisting, heatsetting, and untwisting steps have a very large residual torque. In order to reduce the residual torque, a modified false-twisting method (to be referred to as the two-heater method) in which the yarn is continuously passed between two heaters on a false twisting machine to set the crimps, and a method (to be referred to as the package set method) wherein a cheese of a falsetwisted yarn is heat-treated to set the crimp have been proposed.

According to these methods, there is a close correlation between the bulk and the residual torque of the resulting yarns, and it has been difficult to control the bulk and the residual torque independently of each other. For some applications, it is necessary to reduce the residual torque to substantially zero, or to increase it. However, the realization of this was extremely difficult with the conventional methods.

Methods of reducing the residual torque have been proposed in Japanese Patent Publications Nos. 16,688/64, 28,260/68, and 72,20/71.

The specification of Japanese Patent Publication No. 16,688/64 proposes the production of a bulky yarn that can be handled in the form of a single yarn by using a contact heater having a curved surface in the re-heating process and passing the yarn between a first hollow spindle and a second hollow spindle. By this method, however, sufficient bulkiness cannot be imparted to the yarns.

The method disclosed in the specification of Japanese Patent Publication No. 28,260/68 comprises falsetwisting and heat-setting at least two yarns doubled with each other, applying to the yarns after passage of a falsetwisting spinner a weak twist in a direction opposite to the false-twisting direction before they reach a twist-setting pin or a spreading pin, re-heatsetting the bundle of yarns at this point, and then spreading the bundle yarn into the individual yarns. This method, however, has defects in operation, and since the yarn is treated under tension by the second heater, sufficient bulkiness cannot be imparted to the yarn.

According to Japanese Patent Publication No. 7,220/71, the above-mentioned package setting method is continuously performed. Specifically, a yarn false-twisted by a first heater is treated continuously with heated steam at an overfeed rate of 0 to 30 percent. This, however, has operational difficulties, and cannot reduce the residual torque to the extent achieved by the package set method.

An object of the present invention is to overcome the difficulties of the prior art methods described above, and to provide a novel method of continuously producing bulky synthetic filament yarns whose residual torques have been freely controlled without impairing the bulkiness of the yarns.

According to the present invention, a method is provided of producing a bulky yarn of controlled residual torque, which comprises subjecting a yarn to a series of twisting, heat-setting on a first heater, and untwisting, feeding the yarn into a second heater while rotating it by a fluid nozzle and re-heatsetting the yarn in a second heater, the yarn being maintained in a substantially relaxed condition during the rotation by the fluid nozzle and re-heatsetting by a second heater.

The reason why a yarn which has been subjected to the steps of twisting, heat-setting, and untwisting has a residual torque is that the yarn has the propensity to return to the state at the time of heatsetting. Similarly, the yarn rotated at the time of re-heatsetting tends to return to the state at the time of re-heating after untwisting. Therefore, generally, when the twisting direction at the time of a first heat-setting is opposite to the torque direction of a second heat-setting, the residual torque is balanced, and the yarn has a reduced residual torque and becomes a so-called non-torque crimped yarn free from residual torque. Conversely, when the twisting direction of the first heat-setting is the same as the torque direction of the second heat-setting, the residual torque of the yarn increases to give a crimped yarn useful as creped woven fabrics such as de' chin.

While a reduction in crimpability has been a problem in the conventional two-heater method, this has been solved by the present invention using a fluid nozzle capable of twisting the yarn in a relaxed condition, whereby at the time of the second heat-setting, it is possible to heat-set the crimped yarn without stretching—therefore in a condition in which sufficient bulk can be developed. Accordingly, the present invention provides a bulky yarn of increased torque capable of being applied to non-torque or de' chin, etc.

The preferred embodiment of the present invention will be described with reference to the accompanying drawings in which:

FIG. 1 is a schematic view illustrating the entire process of the method of the present invention;

FIG. 2 is a sectional view showing one embodiment of the fluid nozzle;

FIG. 3 is a view illustrating the relative positions of the second heater, fluid nozzle and twist-nipping point;

FIGS. 4-7 show vertical views of preferred embodiments of a second heater used in the invention.

FIGS. 8-11 show end views of FIGS. 4-7, respectively.

One example of the entire process of the invention will be described with reference to FIG. 1.

Referring to FIG. 1, a starting yarn 2 is withdrawn from a bobbin 1 by a pair of feed rollers 3, and deliv-

ered onto a first heater 4. The yarn is twisted by a spindle 5, and subjected to a first heat-setting by the first heater 4. The yarn is delivered onto a second heater 7 by first delivery rollers 6 while overfeeding. At the time of re-heatsetting by the second heater, the yarn is rotated by a fluid nozzle 8, delivered by second delivery rollers 9, and then wound up on a cheese 11 by a wind-up roller 10 to thereby provide the intended product. In this process, the yarn must be naturally or forcedly cooled between the outlet of the first heater 4 and the spindle 5, and between the outlet of the second heater 7 and the second delivery roller 9.

As a twist-nipping point in re-heatsetting, the first delivery rollers 6 and the second delivery rollers 9 are helpful. The step of twisting, heat-setting on the first heater, and untwisting can be performed by any known method.

The most characteristic feature of the method of the present invention is that a yarn which has been subjected to such twisting, first heatsetting and untwisting is fed to the second heater while being rotated by a fluid nozzle, and during this time, the yarn is maintained in a substantially relaxed condition. This substantially relaxed condition means that a tension in excess of 0.070 g/denier is not exerted on the running yarn. The application of a tension not in excess of 0.050 g/denier is preferred, and most preferably, the tension should not exceed 0.025 g/denier. In order to realize such low tension, it is necessary to adjust the overfeed rate of the yarn to the second heater to above 4 percent. The preferred overfeed rate is at least 6 percent, and more preferably, it is at least 10 percent. There is no particular upper limit of the overfeed rate, but from the standpoint of operation efficiency, it is usually 60 percent, preferably 50 percent, and more preferably 40 percent. Thus, without reducing the bulkiness intended by the present invention, it is possible to obtain a yarn having a freely controlled residual torque with great ease.

In order to maintain the yarn in a substantially relaxed condition, the use of a fluid nozzle and the avoiding of a full contact of the running yarn with the wall surface of the second heater are required in the present invention.

The fluid nozzle has a function of introducing a stream of fluid in the non-axial direction into a twisting path and bringing it into direct collision with a filament yarn which has been fed into the twisting path and is moving at high speed under low tension, eccentrically with respect to the longitudinal axis of the yarn, to thereby give twists to the yarn. Fluid nozzles *per se* based on such theory have previously been used for twisting yarns, and are well known. These fluid nozzles differ somewhat in structure, but all of them can be used in the present invention. Several of the preferred fluid nozzles are disclosed in Japanese Patent Publications Nos. 11,348/61, 11,349/61, 11,350/61 and 11,266/62. Of these, the nozzles disclosed in Japanese Patent Publications No. 11,266/62 are especially preferred, and has the structure as shown in FIG. 2.

Referring to FIG. 2, a fluid introduced from a fluid inlet 12 enters a hollow portion 15 of a main nozzle body 14. The hollow portion 15 is provided eccentrically with a flow passageway 13, so that the fluid which has flowed into the hollow portion 15 is rotated. The rotating direction can be freely changed by changing the position of the flow passageway 13.

The fluid nozzle may be provided before or after the second heater. Generally, it is preferred to provide it after the second heater in view of the installation space of the nozzle and the lowering of the temperature of the heater due to the inflow of the fluid.

Examples of the fluid that can be used in the present invention are inert gases such as nitrogen, neon, crypton, argon, helium, carbon dioxide gas, or air, and steam or water. Because of availability and ease of handling, air is preferably used. The pressure of the fluid can vary according to the kind of fluid, the structure of the fluid nozzle, and the desired torque, but is generally in the range of about 0.05 kg/cm<sup>2</sup> (gauge) to 2.0 kg/cm<sup>2</sup> (gauge).

The second heater used in the invention is of any type which can maintain the yarn in a relaxed condition within the heater and does not permit the full contact of the yarn with the heater. Examples of the second heater include pipe heaters in which the yarn path is

20 hollow, slit type heaters in which the yarn path is a slit-like opening in the direction of yarn travel, or heaters of the type wherein a yarn guiding wire or plate is secured to a desired place on the curved surface in the direction of yarn travel so as to avoid the full contact 25 of the yarn with the heater. Generally, the pipe heaters which are straight in the direction of yarn travel are preferably used.

The full contact type heaters which have previously been used as the second heater cannot attain the substantial relaxed condition as intended in the present invention since the running yarn is held taut due to the contact resistance on their surfaces. In view of this, it is desirable to pass the yarn through the hollow part of the pipe so as to avoid contact with the wall surface of the pipe heater. Smooth industrial operation of such yarn passing is not so easy. If, however, the yarn is contacted only at the inlet and outlet ends of the heater, such operation becomes easy, and the yarn can be maintained in a substantially relaxed condition.

40 The vertical and cross sectional surfaces of the four preferred embodiments of the second heaters are illustrated in FIGS. 4-7 and 8-11, respectively. These heaters are of the type which permit contact of the yarn only at the inlet and outlet ends. In FIGS. 4-7, the

45 heater is shown at 7, and the running yarn at 2. The heaters of FIGS. 4, 5, and 6 do not include a guide for the running yarn, and the heater of FIG. 7 includes guides (16). The positions of contact of the yarn with the heater are indicated by f and f'. The heaters of 50 FIGS. 5 and 6 are obtained by providing the pipe heater 4 with a slit or an opening of larger width, and permit easy yarn stringing operation. Guides can be provided in the heaters of FIGS. 5 and 6 also, as in FIG. 7.

55 The contact positions of the yarn at the inlet and outlet ends of the heater are such that within the inner space of the heater, the yarn does not come into full contact with the wall surface of the heater. For example, when a heater having an inner space with a circular cross section is used, the two contact points should op-

60 pose each other as much as possible. It is however preferred that when the inlet contact point (f) and the outlet contact point (f') are projected on a cross sectional plane perpendicular to the axis of the heater, an angle formed by lines connecting two projected points respectively with the center of the circle is at least 90°, preferably at least 135°, more preferably at least 170°. When these two contact points are selected so as to be

situated opposite to each other, the angle is  $180^\circ$ . The above condition is applicable to a heater of the type wherein the shape of the cross sectional surface of its inner space is an ellipse in which the ratio of the long axis to the short axis is not more than 2.0. While the above discussion has been directed primarily to heaters of circular or elliptical cross section, the shape of the heater is not limited to these shapes. The requirement is that the yarn should not be placed under excessive tension by excessive contact with the wall surface of the heater.

According to the methods involving a fluid nozzle, the yarn is twisted by a rotating stream in the twisting path of the fluid, and therefore, the position of securing the fluid nozzle is important in performing the method of the invention industrially.

It is very desirable that in order to have the rotating ability by the fluid nozzle exhibited effectively and stably and render the residual torque and crimpability of the yarn obtained in each spindle in a multi-spindle operation substantially uniform, the following conditions must be satisfied with respect to the fluid nozzle, the second heater, and the distance and angle between the twist-nipping points. These relations are shown schematically in FIG. 3.

These relations are:

$$l_1 \geq 1.0 \text{ (cm)}$$

$$20^\circ \geq \theta_1 > 0^\circ$$

$$l_2 \leq 30.0 \text{ (cm)}$$

$$20^\circ \geq \theta_2 \geq 0^\circ$$

wherein  $l_1$  is the distance between the outlet contact end of the yarn in the second heater and the center of the fluid nozzle inlet,  $\theta_1$  is an angle formed by the line connecting the outlet contact end with the center of the inlet of the twisting path, and the axial line of the second heater at the outlet contact end,  $l_2$  is the distance between the center of the nozzle twisting path and the twist-setting points, and  $\theta_2$  is an angle formed by the line connecting the center of the nozzle twisting path outlet and the axial line of the nozzle at the outlet center. When woven or knitted fabrics are produced using the yarn obtained under these conditions or such yarn is scoured and dyed, products of very good quality can be obtained. Thus, the method of the present invention is very advantageous industrially.

Furthermore, by employing a fluid nozzle meeting these requirements, the hydrodynamic resistance of the fluid within the fluid nozzle and other yarn twisting portions in contact with yarn guides is very stable and the amount of fluid to be used for giving the same residual torque is also small. Furthermore, the wear of the material of structure on the surface in contact with the yarn is very small, and it is possible to use an inexpensive material of low wear resistance, and it becomes possible to produce a bulky yarn having any desired residual torque with economical advantage.

If the distance ( $l_1$ ) between the outlet of the heater and the nozzle is below 1.0 cm, the residual torque given by the fluid nozzle becomes extremely unstable, and there is a reduced efficiency of operation of passing the yarn through the fluid nozzle, etc. Therefore, the preferred  $l_1$  is at least 1.0 cm, preferably about 1.5 cm. There is no upper limit for  $l_1$  but with increasing  $l_1$ , more space is needed on the falsetwisting machine.

Therefore, the upper limit of the distance is generally 50 cm, preferably 10 cm.

The angle  $\theta_1$  is preferably larger than 0. If the angle  $\theta_1$  is below 0, the residual torque differs greatly from spindle to spindle. On the other hand, if the angle exceeds  $20^\circ$ , the twisting effect by the fluid decreases, and it results in a reduction in crimpability of the yarn. The especially preferred angle  $\theta_1$  is not more than  $15^\circ$ .

If the distance  $l_2$  becomes large, torque effect changes abruptly although differing depending upon the fluid pressure, and there is a setback also with respect to installation space. The advantageous distance  $l_2$  is not more than 30 cm, preferably, not more than 30 cm.

15 The angle  $\theta_2$  is within the range of  $0^\circ$  to  $20^\circ$  for the same reasons as mentioned with respect to the angle  $\theta_2$ .

The Reynolds' number of fluid at the torque twisting portion in the present invention can be very small. By 20 applying a Reynolds' number as small as 1,000 to 5,000, the intended yarn having controlled residual torque can be obtained.

It has been found as a result of a number of experimental results that by applying a Reynolds' number 25 larger than 1,000 and satisfying the following equation when torque is given to the yarn by a fluid nozzle in the direction opposite to the twisting direction in the first step, a yarn of high bulk and substantially free of torque can be produced.

$$30 (-0.0433 T_2 + 15.13) (2.02 \times 10^2) De^{0.200} \geq Re \geq (0.040 T_1 - 0.045 T_2 + 4.2) (0.877 \times 10^2 \times De^{0.366})$$

wherein  $Re$  is Reynolds' number,

$T_1$  is the temperature of the first heatsetting( $^\circ\text{C}$ ),

$T_2$  is the temperature of the second heatsetting( $^\circ\text{C}$ )

De is the denier size of the yarn.

When the Reynolds' number is considerably small, the torque twisting effect is small, and the residual torque in the twisting direction in the first heater is reduced by a fluid nozzle. Therefore, a non-torque bulky yarn cannot be obtained. On the other hand, if the Reynolds' number becomes large, a residual torque is given in the opposite direction in an amount more than the residual torque in the twisting direction on the heater, and the residual torque in the opposite direction increases. As a result, it is impossible to obtain a non-torque bulky yarn. As shown above, the Reynolds' number is affected by the temperature of the first and second heaters, and the denier size of the yarn.

55 The upper limit of the Reynolds' number is not affected by the temperature of the first heater, and is given as a function of the temperature of the second heater and the denier size of the yarn. With increasing heater temperature ( $T_2$ ) and decreasing denier sizes, non-torque bulky yarns can be obtained with smaller Reynolds' number.

On the other hand, the lower limit of the Reynolds' 60 number is given as a function of the temperatures of the first and second heaters, and the denier size of the yarn. Non-torque bulky yarns are obtained with higher temperatures of the first heater, lower temperatures of the second heater, and smaller denier sizes of the yarns. These factors define the lower limit of the Reynolds' number.

65 Such a tendency is readily demonstrated by the fact that in the absence of a fluid nozzle, the residual torque

of a yarn becomes larger with higher temperatures of the first heater and lower temperatures of the second heater; and conversely that it is smaller with lower temperatures of the first heater and higher temperatures of the second heater.

The especially preferred range of Reynolds' number applicable to the production of the non-torque yarns is expressed by the following equations.

$$Re > 1,000$$

$$(-0.0450I_2 + 14.90)(2.89 \times 10^2)De^{0.128} \geq Re \geq (0.025T_1 - 0.0450T_2 + 8.40)(2.08 \times 10^2)De^{0.194}$$

Generally, the temperature of the heater can be expressed by the surface temperature in the case of the contact-type heaters, and by the temperature of the gas phase part in the case of the non-contact type heaters. However, temperature distribution sometimes occurs in the direction of the yarn travel in the heater according to some heating methods using the heaters. For example, in the case of heating with steam or heat-media, such temperature distribution relatively seldom occurs, and the temperature distribution is substantially uniform. On the other hand, in the case of electrical heating, considerable temperature distribution occurs, and therefore, the temperature of the heater should be expressed by an area average temperature in the direction of the travel of the yarn. Generally, it can be simply expressed by the temperature of the central part of the heater.

The filament yarns used in the present invention are thermoplastic synthetic fibers. Among them, polyester, polyamide, polyolefin, polyacrylonitrile, and acetate yarns are advantageously employed either alone or in combination. The method of the present invention is especially advantageously applied to polyamide and polyester yarns, especially polyethylene terephthalate and poly- $\epsilon$ -caproamide yarns, or mixtures of these yarns.

The thermoplastic filament yarns used in the invention may be any filament yarn such as monofilaments or multifilaments although differing somewhat with denier size. Generally, the method of the invention is advantageously applied to multifilaments. The denier size of the useful filament yarn is 15 to 300 denier, preferably 50 to 200 denier, more preferably 70 to 150 denier.

The temperatures of the first and second heaters may be above the glass transition point up to the melting point of the yarn, preferably from about 160° C. up to the melting point. In the case of a polyethylene terephthalate yarn, temperatures in the range of 160° to 230° C. can be effectively employed. The temperature of each heater can be chosen according to the desired bulkiness.

The effective heat-treating time at the heater differs depending upon the type, denier size and number of filaments of the thermoplastic synthetic filament yarn used and the performance of the heater and heating method. Generally, it is at least 0.2 second, preferably at least 0.3 second, especially preferably at least 0.4 second. There is no upper limit, but for economical reasons, the upper limit is usually set at about 3 seconds, preferably about 1.5 second, especially preferably about 1 second. Accordingly, the first and second heaters can be chosen so that they satisfy the effective heat-treating time requirements mentioned above. The

length of each heater can therefore be one which meets such conditions. These conditions are applicable both to the first and second heaters.

In a cooling zone after the first heater and the second heater, the yarn is preferably cooled below the glass transition temperature of the yarn. Since the fluid nozzle mentioned above is used in the present invention, heat dissipation from the yarn achieved by the rotating fluid can be effectively facilitated, and therefore, a much larger cooling effect can be achieved than natural cooling.

The number of twists in the first step twisting is defined generally by the Heberlein's equation disclosed in British Pat. No. 890,992 or the Koechlin's equation although differing according to the end use of the product yarn. For example, the number of twist T [T/M] is given by the following equation

$$T = \alpha C / \sqrt{De}$$

wherein  $\alpha$  is a twist coefficient,  $C$  is a constant determined by the yarn material such as polyethylene terephthalate or poly- $\epsilon$ -caproamide, and  $De$  is the denier of the yarn. The twist coefficient is 0.5 to 1.10, preferably from 0.80 to 1.05.

On the other hand, there is no particular limitation on the speed of the running yarn. Although different according to the type of the false-twister, processing conditions, and the yarn, the speed is usually 60 meters per minute or above. The upper limit is automatically set according to the above-mentioned conditions.

The direction of yarn travel is not particularly limited (e.g., the yarn can be travelled upwardly, downwardly, or even horizontally).

The invention will be described further by the following Examples and Comparative Examples.

In the Examples, the residual torque is the number of twists of a yarn at a time when a load of 2 mg per denier is applied to the yarn and the yarn stops rotating. The measured value is one per 25 cm, and the rotating force in the Z direction is positive.

The crimp shrinkage is measured as follows:

The length ( $l_0$ ) of a yarn is measured under a load of 202 mg/de, and then the yarn is treated with boiling water for 20 minutes under a load of 2 mg/de. The yarn is spontaneously dried for one day and night in the absence of load, and then the length ( $l_1$ ) is measured under a load of 202 mg/de. Then under a load of 2 mg/de, the length ( $l_2$ ) of the yarn is measured. The crimp shrinkage is expressed by the following equation.

$$\text{Crimp shrinkage} = l_1 - l_2 / l_0 \times 100 (\%)$$

If the yarn is a poly- $\epsilon$ -caproamide yarn, the heavier load used is 102 mg/de instead of 202 mg/de.

#### EXAMPLES 1 TO 8

A 150-denier/30 filament semidull yarn of polyethylene-terephthalate was crimped at an overfeed rate of 4 percent, and a yarn speed of 125 meters/min. in the productional process shown in FIG. 1. The number of false twists was 2670 (T/M), and the false-twisting direction Z. The heater used was a curved surface contact type (heater length 1 m) was a heating temperature of the first heater being adjusted to 220° C. Then, the yarn was passed through the second heater and the center of the fluid nozzle at an overfeed rate of 17 percent. The second heater is a pipe type having a circular

vertical section in axial direction. The heating temperature of the second heater was 220° C., and the heater length was 50 cm. The fluid nozzle used was of the type shown in FIG. 2 which rotated in the S direction. As the fluid, air was used, and the pneumatic pressure at the inlet 13 of the nozzle was adjusted as indicated in Table 1. The results are also shown in Table 1.

Table 1

| Examples | Pneumatic Pressure(kg/cm <sup>2</sup> G) | Residual torque (T/0.25 m) | Crimp Shrinkage (%) |
|----------|------------------------------------------|----------------------------|---------------------|
| 1        | 0                                        | 33                         | 16.5                |
| 2        | 0.10                                     | 4                          | 16.9                |
| 3        | 0.20                                     | -13                        | 16.4                |
| 4        | 0.30                                     | -25                        | 16.2                |
| 5        | 0.40                                     | -32                        | 16.0                |
| 6        | 0.50                                     | -40                        | 15.9                |
| 7        | 0.60                                     | -44                        | 15.9                |
| 8        | 0.70                                     | -47                        | 15.5                |

It is seen from the results of Table 1 that irrespective of the crimp shrinkage, the residual torque can be freely controlled. By increasing the pneumatic pressure, the residual torque in the Z direction becomes small, and the residual torque is balanced between the pneumatic pressures 0.1 kg/cm<sup>2</sup>G and 0.2 kg/cm<sup>2</sup>G, and becomes zero to give a completely non-torque yarn. With further increase in pneumatic pressure, the residual torque increases in the S direction. However, during this time, the residual torque changed greatly, but the crimp shrinkage hardly changed.

#### EXAMPLE 9 AND COMPARATIVE EXAMPLES 1, 2 AND 3

The procedure of Example 1 was repeated except that the overfeed rate was 3 percent, the yarn speed was 105 meters/min., the number of twist of 2,500 (T/M), the temperature of the first heater was 210° C., the temperature of the second heater was 215° C., the second overfeed rate was 20 percent, and the pneumatic pressure was 0.12 kg/cm<sup>2</sup>G. For comparative purposes, the fluid nozzle was removed in the above Example, and the yarn was simply heat-set on the second heater (comparative Example 1); a hollow spindle was provided in place of the fluid nozzle 5, and also a contact heater was provided (the number of false twist 2040 (T/M), the false-twisting direction S, the temperature of the second heater 205° C., and the second overfeed rate 2 percent) (Comparative Example 2); and the overfeed rate was adjusted to 6 percent in Comparative Example 2 (comparative Example 3). The properties of the treated yarns and their tension at the outlet of the second heater were compared as shown in Table 2 below.

Table 2

|            | Residual torque | Crimp shrinkage | Tension (g/de) | Remarks                                                   |
|------------|-----------------|-----------------|----------------|-----------------------------------------------------------|
| Example 9  | 4               | 15.4            | 0.020          |                                                           |
| Comp. Ex.1 | 35              | 16.3            | 0.017          |                                                           |
| Comp. Ex.2 | 8               | 7.2             | 0.080          |                                                           |
| Comp. Ex.3 | —               | —               | —              | Yarn breakage frequent; impossible to continue processing |

As is seen from Table 2, there is no substantial difference in crimp shrinkage between Example 9 and Comparative Example 1, but a drastic difference in residual torque is observed between them. In Example 9, a substantially nontorque yarn was obtained, whereas the yarn obtained in Comparative Example 2 has a large residual torque.

Furthermore, it is seen that in Comparative Example 2, the residual torque of the residual torque was reduced in the yarn of Comparative Example 2, but the crimp shrinkage is half as low as that of the yarn of Example 9.

The bulky yarn according to the present invention has a markedly reduced residual torque as compared with the conventional method, and its bulkiness is almost the same as that of the conventional bulky yarns. Therefore, when the yarn of the present invention is used for knitting, snarls do not occur. The knittability of the yarn obtained by the invention is very good, and the final knitted product obtained has great bulkiness.

#### EXAMPLE 10 AND COMPARATIVE EXAMPLE 4

The procedure of Example 1 was repeated except that a polyethylene-terephthalate yarn (Semi Dull) of 50 denier and 24 filaments was used, the first overfeed rate was 5 percent, the yarn speed was 85 meters/min., the number of twists was 3900 (T/M), the false-twisting direction was Z (S), the temperature of the first heater was 220° C., the second overfeed rate was 15 percent, the temperature of the second heater was 180° C., and a fluid nozzle capable of rotating the yarn in the same direction as the false-twisting direction [the yarn rotating direction Z (S)], and the pneumatic pressure was 0.4 kg/cm<sup>2</sup>G.

For comparative purpose, the properties of the yarn which had been just subjected to the steps of twisting, heat-setting, and untwisting are shown in Table 3.

Table 3

|                       | Residual torque | Crimp shrinkage |
|-----------------------|-----------------|-----------------|
| Example 10            | 84              | 31.2            |
| Comparative Example 4 | 53              | 35.1            |

It is seen that the bulky yarn obtained according to the present has a remarkably large residual torque and is best suited for application as de' chin, etc.

#### EXAMPLES 11 to 18

The procedure of Example 1 was repeated except that the temperature of the first heater was 205° C., the temperature of the second heater was 220° C., the pneumatic pressure was 0.10 kg/cm<sup>2</sup>G, and the second overfeed rate was changed as shown in Table 4 below. The results are shown in Table 4.

Table 4

| Examples | Second overfeed rate (%) | Tension at the 2nd heater(S/de) | Residual torque | Crimp shrinkage |
|----------|--------------------------|---------------------------------|-----------------|-----------------|
| 11       | 4                        | 0.070                           | 8               | 9.1             |
| 12       | 6                        | 0.050                           | 5               | 10.8            |
| 13       | 8                        | 0.025                           | 4               | 11.7            |
| 14       | 10                       | 0.025                           | 4               | 12.0            |
| 15       | 15                       | 0.025                           | 3               | 12.7            |

Table 4-Continued

| Examples | Second overfeed rate (%) | Tension at the 2nd heater (S/de) | Residual torque | Crimp shrinkage |
|----------|--------------------------|----------------------------------|-----------------|-----------------|
| 16       | 20                       | 0.023                            | 4               | 12.8            |
| 17       | 40                       | 0.020                            | 4               | 12.7            |
| 18       | 50                       | 0.020                            | 4               | 12.9            |

It is seen from Table 4 that with increasing second overfeed rates, the yarn tension at the second heater is reduced, and the yarn can be maintained in a substantially relaxed condition. No remarkable difference in residual torque and crimp shrinkage was observed at this time.

#### COMPARATIVE EXAMPLES 5 TO 8

The procedure of Example 11 was repeated except that the second overfeed rate was changed as shown in Table 5.

Table 5

| Comparative Examples | Second overfeed rate (%) | Tension of the yarn in the second heater | Residual torque | Crimp shrinkage (%) |
|----------------------|--------------------------|------------------------------------------|-----------------|---------------------|
| 5                    | 0                        | 0.293                                    | 18              | 3.5                 |
| 6                    | 1                        | 0.225                                    | 15              | 4.0                 |
| 7                    | 2                        | 0.147                                    | 11              | 5.4                 |
| 8                    | 3                        | 0.086                                    | 9               | 6.8                 |

#### EXAMPLES 19 TO 24

The procedure of Example 11 was repeated except that the yarn speed was 125 meters/min., the second overfeed rate was 17 percent, the yarn was contacted with the second heater only at the inlet and outlet ends as shown in FIGS. 4-7, the angle  $\theta$  shown in FIG. 3, the pneumatic pressure was 0.20 kg/cm<sup>2</sup>G, a fluid nozzle having the same properties was used. The results are shown in Table 6. The symbol  $\bar{x}$  shows a value of arithmetic means of residual torques or crimp shrinkage of 8 spindles, and R indicates the maximum-minimum value.

Table 6

| Examples | $\theta$ (°) | Residual torque<br>$\bar{x}$ | Residual torque<br>R | Crimp shrinkage<br>$\bar{x}$ | Crimp shrinkage<br>R |
|----------|--------------|------------------------------|----------------------|------------------------------|----------------------|
| 19       | 90           | 7.2                          | 10                   | 12.4                         | 1.7                  |
| 20       | 120          | 6.7                          | 9                    | 12.5                         | 1.5                  |
| 21       | 135          | 6.4                          | 7                    | 12.4                         | 1.0                  |
| 22       | 165          | 6.3                          | 6                    | 12.6                         | 0.9                  |
| 23       | 170          | 6.2                          | 5                    | 12.8                         | 0.6                  |
| 24       | 180          | 6.2                          | 5                    | 12.8                         | 0.6                  |

The yarn obtained was knitted on a 18-gauge circular knitting machine, and then scoured and dyed. The product had good surface condition and feeling and no dyeing unevenness was observed.

#### COMPARATIVE EXAMPLE 9

The procedure of Example 19 was repeated except that a guide and a fluid nozzle were provided at the second heater so that they passed through the center of the heater. The resulting yarn had a residual torque of 3.3 ( $\bar{x}$ ) and 35 (R). There was a marked deviation in residual torque among the spindles.

#### COMPARATIVE EXAMPLES 10 TO 12

The procedure of Example 19 was repeated except that  $\theta$  was changed as indicated in Table 7. The results are shown in Table 7.

Table 7

| Comparative Examples | $\theta$ | Residual torque<br>$\bar{x}$ | Residual torque<br>R | Crimp shrinkage<br>$\bar{x}$ | Crimp shrinkage<br>R |
|----------------------|----------|------------------------------|----------------------|------------------------------|----------------------|
| 10                   | 0        | 21.3                         | 22                   | 10.6                         | 2.5                  |
| 11                   | 45       | 9.6                          | 15                   | 11.5                         | 2.3                  |
| 12                   | 80       | 7.9                          | 11                   | 12.0                         | 1.9                  |

#### EXAMPLES 25 AND 26

The procedure of Example 19 was repeated except that a polyethylene-terephthalate yarn (semidull; 50 denier/24 filaments) was crimped at a first overfeed rate of 5 percent, and a yarn speed of 85 meters/min. with the number of false-twists of 3,900 T/M in the S direction while the temperature of the first heater was being maintained at 220° C.; and subsequently, the crimped yarn was treated in the same way as in Example 19 at a second overfeed rate of 15 percent and a pneumatic pressure at the nozzle of 0.4 kg/cm<sup>2</sup>G while the temperature of the second heater was being maintained at 180° C. (yarn rotating direction S; the angle was changed as indicated in Table 8).

Table 8

| Examples | $\theta$ (°) | Residual torque<br>(times/0.25 M)<br>$\bar{x}$ | Residual torque<br>R | Crimp shrinkage (%)<br>$\bar{x}$ | Crimp shrinkage (%)<br>R |
|----------|--------------|------------------------------------------------|----------------------|----------------------------------|--------------------------|
| 25       | 135          | 81                                             | 10                   | 35.0                             | 1.5                      |
| 26       | 180          | 84                                             | 8                    | 35.1                             | 1.0                      |

#### COMPARATIVE EXAMPLES 13 AND 14

The procedure of Example 25 was repeated except that the angle was changed as shown in Table 9. The results obtained are shown in Table 9.

Table 9

| Comparative Examples | Angle $\theta$ | Residual torque<br>(times/1.25M) |    | Crimp shrinkage (%) |      |
|----------------------|----------------|----------------------------------|----|---------------------|------|
|                      |                | $\bar{x}$                        | R  | $\bar{x}$           | R    |
| 50                   | 13             | 45                               | 69 | 18                  | 33.1 |
|                      | 14             | 80                               | 78 | 11                  | 34.2 |

#### EXAMPLES 27 TO 42

The procedure of Example 24 was repeated except as noted below:

The second heater: a pipe heater provided with guides at its inlet and outlet such as shown in FIG. 7

The temperature of the second heater: 215° C.

The distance  $l_1$  (cm): as shown in Table 10 in FIG. IV

The angle  $\theta_1$  (°): as shown in Table 10

The distance  $l_2$ : 4.0 cm between the center of the nozzle

The fluid nozzle: provided at the position at which the angle is 0.

The results obtained are shown in Table 10 below.

Table 10

| Examples | $l_1$ (cm) | $\theta_1$ (°) | Residual torque( $\bar{x}$ ) | Tension of yarn at second heater |
|----------|------------|----------------|------------------------------|----------------------------------|
| 27       | 1.0        | 5              | 10.4                         | 0.020                            |
| 28       | 1.0        | 10             | 10.8                         | 0.022                            |
| 29       | 1.0        | 15             | 10.6                         | 0.021                            |
| 30       | 1.0        | 20             | 13.4                         | 0.021                            |
| 31       | 1.5        | 5              | 9.5                          | 0.020                            |
| 32       | 1.5        | 10             | 9.8                          | 0.018                            |
| 33       | 1.5        | 15             | 10.0                         | 0.019                            |
| 34       | 1.5        | 20             | 11.6                         | 0.020                            |
| 35       | 3.0        | 5              | 9.4                          | 0.018                            |
| 36       | 3.0        | 10             | 9.2                          | 0.019                            |
| 37       | 3.0        | 15             | 9.7                          | 0.018                            |
| 38       | 3.0        | 20             | 11.9                         | 0.020                            |
| 39       | 3.8        | 5              | 8.2                          | 0.020                            |
| 40       | 3.8        | 10             | 8.7                          | 0.020                            |
| 41       | 3.8        | 15             | 8.5                          | 0.018                            |
| 42       | 3.8        | 20             | 8.9                          | 0.020                            |

## COMPARATIVE EXAMPLES 15 TO 24

The procedure of Example 27 was repeated except that the distance  $l_1$  and the angle  $\theta_2$  were changed as shown in Table 11. The results obtained are shown in Table 11.

Table 13

| Examples | Distance ( $l_2$ ) (cm) | Residual torque( $\bar{x}$ ) |
|----------|-------------------------|------------------------------|
| 5        | 47                      | 10                           |
|          | 48                      | 15                           |
|          | 49                      | 20                           |
|          | 50                      | 30                           |

## 10 COMPARATIVE EXAMPLES 25 AND 26

The procedure of Example 47 was repeated except that the distance  $l_2$  was changed as shown in Table 14. The results are shown in Table 14.

## 15 Table 14

| Comparative Examples | Distance $l_2$ (cm) | Residual torque( $\bar{x}$ ) |
|----------------------|---------------------|------------------------------|
| 25                   | 35                  | -1.3                         |
| 26                   | 40                  | -10.2                        |

## EXAMPLES 51 TO 55

The procedure of Example 36 was repeated except

Table 11

| Comparative Examples | $l_1$ (cm) | $\theta_1$ (°) | Residual torque( $\bar{x}$ ) | Tension at the second heater (gr/de) | Remarks                   |
|----------------------|------------|----------------|------------------------------|--------------------------------------|---------------------------|
| 15                   | 0.8        | 5              | 12.3                         | 0.024                                | Rotation of yarn unstable |
| 16                   | 1.0        | 0              | -1.0                         | 0.016                                |                           |
| 17                   | 1.0        | 25             | 13.7                         | 0.023                                |                           |
| 18                   | 1.0        | 30             | 17.8                         | 0.025                                |                           |
| 19                   | 3.0        | 0              | 3.8                          | 0.017                                |                           |
| 20                   | 3.0        | 25             | 13.4                         | 0.022                                |                           |
| 21                   | 3.0        | 30             | 17.9                         | 0.025                                |                           |
| 22                   | 3.8        | 0              | 8.5                          | 0.017                                |                           |
| 23                   | 3.8        | 25             | 13.3                         | 0.020                                |                           |
| 24                   | 3.8        | 30             | 16.4                         | 0.022                                |                           |

## EXAMPLES 43 TO 46

The procedure of Example 27 was repeated except that the distance  $l_1$  was 3.0 cm, the angle  $\theta_1$  was 10°, and the pneumatic pressure was changed as indicated in Table 12. The results obtained are shown in Table 12.

Table 12

| Examples | Pneumatic pressure(kg/cm <sup>2</sup> G) | Residual torque (twist/0.25 m)( $\bar{x}$ ) |
|----------|------------------------------------------|---------------------------------------------|
| 43       | 0.15                                     | 20.9                                        |
| 44       | 0.25                                     | -0.4                                        |
| 45       | 0.30                                     | -13.0                                       |
| 46       | 0.40                                     | -25.0                                       |

## EXAMPLES 47 TO 50

The procedure of Example 43 was repeated except that the pneumatic pressure was 0.20 kg/cm<sup>2</sup>G, and the distance was changed as shown in Table 13. The results are shown in Table 13.

that the angle was varied as shown in Table 15. The results are shown in Table 15.

## Table 15

| Example | $\theta_2$ (°) | Residual torque( $\bar{x}$ ) | Tension at the second heater (gr/de) |
|---------|----------------|------------------------------|--------------------------------------|
| 51      | 0              | 7.8                          | 0.017                                |
| 52      | 5              | 9.2                          | 0.018                                |
| 53      | 10             | 9.6                          | 0.020                                |
| 54      | 15             | 9.6                          | 0.020                                |
| 55      | 20             | 10.2                         | 0.021                                |

## COMPARATIVE EXAMPLES 27 AND 28

The procedure of Example 36 was repeated except that the angle  $\theta_2$  was changed as shown in Table 16. The results are shown in Table 16.

## Table 16

| Comparative Examples | $\theta_2$ (°) | Residual torque( $\bar{x}$ ) | Tension at second heater (g/de) |
|----------------------|----------------|------------------------------|---------------------------------|
| 27                   | 25             | 13.2                         | 0.023                           |
| 28                   | 30             | 17.5                         | 0.025                           |

## EXAMPLES 56 TO 67

The procedure of Examples 36 was repeated except as noted below:

1. Temperature of the first heater was 220° C.
2. Temperature of the second heater was changed as shown in Table 17.
3. The ratio of the sectional area of the twisting path to that of a fluid flow was 11:1.
4. The diameter of the twisting path was 2.5 mm.
5. The fluid stream intersects the twisting path in a direction at right angles to the path and flows in a tangential direction with respect to the twisting path.
6. A fluid nozzle of the type shown in FIG. 2 was used, and by changing the air velocity, the Reynolds' number in the twisting path of the fluid nozzle was changed as shown in Table 17.

Table 17

| Examples | Temperature of second heater | Reynolds' number | Residual torque | Crimp shrinkage |
|----------|------------------------------|------------------|-----------------|-----------------|
| 56       | 220°C.                       | 1,800            | 18              | 16.8            |
| 57       | 220                          | 2,500            | 1               | 16.5            |
| 58       | 220                          | 3,000            | -19             | 16.1            |
| 59       | 200                          | 2,500            | 16              | 21.3            |
| 60       | 200                          | 3,000            | -2              | 21.0            |
| 61       | 200                          | 3,300            | -15             | 19.8            |
| 62       | 180                          | 2,750            | 15              | 25.4            |
| 63       | 180                          | 3,000            | 4               | 25.2            |
| 64       | 180                          | 3,500            | -16             | 24.8            |
| 65       | 160                          | 3,200            | 18              | 27.5            |
| 66       | 160                          | 3,750            | 0               | 27.1            |
| 67       | 160                          | 4,250            | -13             | 26.4            |

## COMPARATIVE EXAMPLES 29 TO 40

The procedure of Example 56 was repeated except that the temperature of the second heater and the Reynolds' number were changed as indicated in Table 18. The results are shown in Table 18. The Reynolds' numbers in these Comparative Examples were outside the scope of the present invention.

Table 18

| Comparative Examples | Temperature of second heater | Reynolds' number | Residual torque | Crimp shrinkage |
|----------------------|------------------------------|------------------|-----------------|-----------------|
| 29                   | 220°C.                       | 0                | 31              | 16.4            |
| 30                   | 220                          | 1,000            | 28              | 16.6            |
| 31                   | 220                          | 3,500            | -34             | 13.5            |
| 32                   | 200                          | 0                | 32              | 20.3            |
| 33                   | 200                          | 1,000            | 31              | 21.0            |
| 34                   | 200                          | 3,750            | -30             | 19.2            |
| 35                   | 180                          | 0                | 36              | 24.1            |
| 36                   | 180                          | 1,000            | 34              | 24.4            |
| 37                   | 180                          | 4,000            | -34             | 25.0            |
| 38                   | 160                          | 0                | 38              | 26.2            |
| 39                   | 160                          | 1,000            | 36              | 26.5            |
| 40                   | 160                          | 5,000            | -32             | 25.8            |

## EXAMPLES 68 TO 79

The procedure of Example 56 was repeated except that the temperature of the first heater was adjusted to 200° C., and the temperature of the second heater and the Reynolds' number were changed as shown in Table 19. The Reynolds' numbers were all within the scope of the present invention.

Table 19

| Examples | Temperature of second heater | Reynolds' number | Residual torque | Crimp shrinkage |
|----------|------------------------------|------------------|-----------------|-----------------|
| 68       | 220°C.                       | 1,500            | 18              | 11.2            |
| 69       | 220                          | 2,250            | 2               | 11.5            |
| 70       | 220                          | 2,700            | -12             | 11.1            |
| 71       | 200                          | 2,000            | 19              | 15.2            |
| 72       | 200                          | 2,750            | 2               | 14.8            |
| 73       | 200                          | 3,250            | -10             | 14.5            |
| 74       | 180                          | 2,500            | 16              | 20.2            |
| 75       | 180                          | 3,250            | 1               | 19.0            |
| 76       | 180                          | 3,750            | -15             | 18.4            |
| 77       | 160                          | 3,250            | 13              | 21.5            |
| 78       | 160                          | 3,750            | -1              | 21.7            |
| 79       | 160                          | 4,250            | -15             | 20.8            |

## COMPARATIVE EXAMPLES 41 TO 52

The procedure of Example 68 was repeated except that the temperature of the second heater and the Reynolds' number were changed as shown in Table 20. The results are shown in Table 20. The Reynolds' numbers were all outside the scope of the present invention.

Table 20

| Comparative Examples | Temperature of second heater (°C.) | Reynolds' number | Residual torque | Crimp shrinkage |
|----------------------|------------------------------------|------------------|-----------------|-----------------|
| 41                   | 220                                | 0                | 24              | 10.0            |
| 42                   | 220                                | 1,000            | 23              | 10.6            |
| 43                   | 220                                | 3,500            | -34             | 10.3            |
| 44                   | 200                                | 0                | 28              | 14.1            |
| 45                   | 200                                | 1,000            | 26              | 14.4            |
| 46                   | 200                                | 4,000            | -32             | 13.5            |
| 47                   | 180                                | 0                | 31              | 18.5            |
| 48                   | 180                                | 1,000            | 28              | 18.8            |
| 49                   | 180                                | 4,250            | -31             | 18.0            |
| 50                   | 160                                | 0                | 36              | 20.5            |
| 51                   | 160                                | 1,000            | 34              | 20.8            |
| 52                   | 160                                | 4,750            | -30             | 20.1            |

## EXAMPLES 80 TO 85

The procedure of Example 56 was repeated except that the temperature of the second heater was adjusted to 205° C., and the Reynolds' number and the second overfeed rate were changed as shown in Table 12. The Reynolds' numbers were all within the scope of the present invention. The results are shown in Table 21.

Table 21

| Examples | Second overfeed rate | Reynolds' number | Residual torque | Crimp shrinkage |
|----------|----------------------|------------------|-----------------|-----------------|
| 80       | 8 %                  | 2,500            | 12              | 11.7            |
| 81       | 8                    | 3,000            | -11             | 10.8            |
| 82       | 25                   | 2,500            | 17              | 12.6            |
| 83       | 25                   | 2,000            | -14             | 12.3            |
| 84       | 50                   | 2,500            | 15              | 12.8            |
| 85       | 50                   | 3,000            | -15             | 12.7            |

## EXAMPLES 68 TO 79

The procedure of Example 56 was repeated except that the second overfeed rate was 17 percent, and the temperature of the second heater, the speed of the yarn

and the Reynolds' number were changed as shown in Table 22. The results obtained are shown in Table 22. The Reynolds' numbers were all within the scope of the present invention.

Table 22

| Examples | Yarn speed at the inlet of feed roller (meters/min.) | Reynolds's number | Residual torque | Crimp Shrinkage |
|----------|------------------------------------------------------|-------------------|-----------------|-----------------|
| 86       | 85                                                   | 2,500             | 12              | 13.3            |
| 87       | 85                                                   | 3,000             | -18             | 13.7            |
| 88       | 105                                                  | 2,500             | 9               | 12.4            |
| 89       | 105                                                  | 3,000             | -18             | 12.6            |

## Examples 90 TO 98

The procedure of Example 80 was repeated except that the polyethylene-terephthalate yarn (Semi-dull), the temperatures of the first and second heaters, the number of twists, and the Reynolds' number were changed as indicated in Table 23. The Reynolds' number were all within the scope of the present invention. The results obtained are shown in Table 23.

Table 23

| Exam-<br>ples | Denier | Number<br>of<br>fila-<br>ments | Temper-<br>ature<br>of<br>first<br>heater | Temper-<br>ature<br>of<br>second<br>heater | Number<br>of<br>twists | Reynolds<br>number | Resi-<br>dua<br>l<br>torque | Crimp<br>shrin-<br>kage |
|---------------|--------|--------------------------------|-------------------------------------------|--------------------------------------------|------------------------|--------------------|-----------------------------|-------------------------|
| 90            | 125    | 24                             | 212                                       | 220                                        | 3070                   | 2500               | 10                          | 12.4                    |
| 91            | 125    | 24                             | 212                                       | 220                                        | 3070                   | 2750               | 0                           | 12.2                    |
| 92            | 125    | 24                             | 212                                       | 220                                        | 3070                   | 3000               | -11                         | 12.6                    |
| 93            | 100    | 24                             | 215                                       | 220                                        | 2950                   | 2500               | 16                          | 11.6                    |
| 94            | 100    | 24                             | 215                                       | 220                                        | 2950                   | 2750               | 7                           | 11.4                    |
| 95            | 100    | 24                             | 215                                       | 220                                        | 2950                   | 3000               | -4                          | 11.1                    |
| 96            | 75     | 24                             | 215                                       | 200                                        | 3370                   | 2750               | 12                          | 13.7                    |
| 97            | 75     | 24                             | 215                                       | 200                                        | 3370                   | 3000               | 2                           | 13.2                    |
| 98            | 75     | 24                             | 215                                       | 200                                        | 3370                   | 3250               | -10                         | 13.0                    |

## COMPARATIVE EXAMPLES 53 TO 58

The procedure of Example 80 was repeated except that the polyethylene-terephthalate yarn (Semi-dull), the temperatures of the first and second heaters, the number of twists, and the Reynolds number were changed as indicated in Table 24. The Reynolds' numbers were all outside the scope of the present invention. The results obtained are shown in Table 24.

Table 24

| Compar-<br>ative<br>Exam-<br>ples | Denier | Number<br>of<br>fila-<br>ment | Temper-<br>ature<br>of<br>first<br>heater | Temper-<br>ature<br>of<br>second<br>heater | Number<br>of<br>twists | Reynolds<br>number | Resi-<br>dua<br>l<br>torque | Crimp<br>shrin-<br>kage |
|-----------------------------------|--------|-------------------------------|-------------------------------------------|--------------------------------------------|------------------------|--------------------|-----------------------------|-------------------------|
| 53                                | 125    | 24                            | 212                                       | 220                                        | 3070                   | 1000               | 28                          | 11.7                    |
| 54                                | 125    | 24                            | 212                                       | 220                                        | 3070                   | 3500               | 30                          | 12.4                    |
| 55                                | 100    | 24                            | 215                                       | 220                                        | 2960                   | 1000               | 32                          | 11.6                    |
| 56                                | 100    | 24                            | 215                                       | 220                                        | 2960                   | 3500               | -27                         | 11.0                    |
| 57                                | 75     | 24                            | 215                                       | 200                                        | 3370                   | 1000               | 40                          | 13.6                    |
| 58                                | 75     | 24                            | 215                                       | 200                                        | 3370                   | 3750               | -34                         | 13.0                    |

## EXAMPLES 99 TO 101

The procedure of Example 72 was repeated except that the diameter of the twisting path was changed as indicated in Table 25. The Reynolds' numbers were all

within the scope of the present invention. The results obtained are also shown in Table 25.

Table 25

| 5<br>Examples | Diameter of twisting path (mm) | Residual torque | Crimp shrinkage |
|---------------|--------------------------------|-----------------|-----------------|
| 99            | 2.0                            | 4               | 14.9            |
| 100           | 3.0                            | 0               | 14.7            |
| 101           | 5.0                            | -2              | 15.0            |

## EXAMPLES 102 AND 103

The procedure of Example 72 was repeated except that the fluids shown in Table 26 were used instead of air. The Reynolds' numbers were all within the scope of the present invention. The results obtained are shown in Table 26.

Table 26

| 20<br>Examples | Fluids         | Residual torque | Crimp shrinkage |
|----------------|----------------|-----------------|-----------------|
| 102            | Nitrogen       | 3               | 14.6            |
| 103            | Carbon dioxide | 5               | 15.1            |

45 In accordance with the procedure of Example 56, a poly- $\epsilon$ -caproamide yarn (Semi dull 70 denier/24 filaments) was crimped at a first overfeed rate of zero percent and a yarn speed of 100 meters per minute with the number of false twists of 3180 T/M in the Z direction while the temperature of the first heater was main-

50 tained at 160°C. Thereafter, the yarn was treated in the same way as set forth in Example 56 except that the second overfeed rate was changed to 16 percent, the temperature of the first heater was adjusted to 190°C., and the Reynolds' number was set at 2,000. The result-

ing processed yarn had a residual torque of 12 and a crimp shrinkage of 14.1 percent. The Reynolds' number was within the scope of the present invention.

#### COMPARATIVE EXAMPLES 59 AND 60

The procedure of Example 104 was repeated except that the Reynolds' number was changed as shown in Table 27. The results are shown in Table 27. The Reynolds' numbers were all outside the scope of the present invention.

Table 27

| Comparative Examples | Reynolds' number | Residual torque | Crimp shrinkage (%) |
|----------------------|------------------|-----------------|---------------------|
| 59                   | 0                | 48              | 14.4                |
| 60                   | 4,000            | -36             | 12.6                |

#### EXAMPLE 105

The procedure of Example 104 was repeated except that a 50 de/12 fil semi-dull filament yarn of poly-epsilon-caproamide was processed under the following conditions:

First overfeed rate: 0%  
Number of false twists: 3670 T/M  
Second overfeed rate: 10%  
Reynolds' number: 2,000 (within the scope defined in claim 16)

The resulting yarn had a residual torque of 8.

#### THE 106 AND 107 AND COMPARATIVE EXAMPLES 61 AND 62

A 70 de/24 fil semidull yarn was processed under the following conditions:

First overfeed rate: 0%  
Yarn speed: 100 meters/min.  
Number of false twists: 3180 T/M  
False-twisting direction: Z  
Temperature of the first heater: 160°C.  
Temperature of the second heater: 190°C.  
Second overfeed rate: 16%  
Pneumatic pressure: 0.20 kg/cm<sup>2</sup>G

The results obtained are shown in Table 28.

Table 28

| Examples     | $\theta$ | Residual torque |    | Crimp shrinkage |     |
|--------------|----------|-----------------|----|-----------------|-----|
|              |          | $\bar{x}$       | R  | $\bar{x}$       | R   |
| Example 106  | 135      | 1.6             | 8  | 14.0            | 1.0 |
| Example 107  | 180      | 1.0             | 6  | 14.3            | 0.7 |
| Comp. Ex. 61 | 45       | 4.8             | 17 | 13.1            | 3.4 |
| Comp. Ex. 62 | 80       | 3.6             | 11 | 13.5            | 2.3 |

What is claimed is:

1. A method of producing a bulky yarn having a controlled residual torque, which comprises subjecting a thermoplastic synthetic filament yarn to a series of

twisting, heat-setting on a first heater, and untwisting; feeding the yarn into a second heater while rotating said yarn by means of a fluid nozzle; and re-heat-setting said yarn in the second heater, said yarn being maintained in a substantially relaxed state during the rotation by said fluid nozzle and said re-heat-setting by said second heater.

2. The method of claim 1, wherein rotation is imparted to said yarn by means of said fluid nozzle in a direction opposite to the twisting direction to thereby produce a substantially non-torque filament yarn.

3. The method of claim 1, wherein rotation is imparted to said yarn by means of said fluid nozzle in the same direction as the twisting direction to thereby produce a yarn having an increased residual torque.

4. The method of claim 1, wherein said yarn does not come into full contact with the wall surface of said second heater.

5. The method of claim 1, wherein said yarn contacts said second heater only at its inlet and outlet ends.

6. The method of claim 1, wherein the yarn is maintained under a tension lower than 0.070 g/denier during rotation by said fluid nozzle.

7. The method of claim 6, wherein the yarn is maintained under a tension lower than 0.050 g/denier during rotation by said fluid nozzle.

8. The method of claim 7, wherein the yarn is maintained under a tension lower than 0.025 g/denier during rotation by said fluid nozzle.

9. The method of claim 1, wherein said yarn is overfed to said second heater at an overfeed rate maintained at above 4 percent.

10. The method of claim 9, wherein the overfeed rate of the yarn to said second heater is maintained at above 6 percent.

11. The method of claim 10, wherein the overfeed rate of the yarn to said second heater is maintained at above 10 percent.

12. The method of claim 5, wherein the angles of said yarn with respect to the inlet and outlet ends of said second heater are selected so that when the inlet contact point and outlet contact point of said yarn at said second heater are projected on a cross-sectional plane perpendicular to the axis of said heater, the two projected points are connected by an arc of a circle or an ellipse, and an angle formed by connecting said two projected points with the center of said circle or ellipse is at least 90°, and when said arc is a part of the arc of the ellipse, said ellipse has a long axis to short axis ratio of not more than 2.0:1.

13. The method of claim 5, wherein the yarn is treated under the following conditions:

$$l_1 \geq 1.0 \text{ (cm)}$$

$$20^\circ \geq \theta > 0^\circ$$

$$l_2 \leq 30.0 \text{ cm}$$

$$20^\circ \geq \theta_2 \geq 0^\circ$$

60 wherein  $l_1$  is the distance between the point at which said yarn contacts the outlet of said second heater and the point at which the yarn passes to the center of said fluid nozzle inlet multiplied by  $\cos \theta_1$ ;  $\theta_1$  is an angle formed by the line joining the point at which said yarn contacts the outlet of said second heater with the point at which the yarn passes to the center of inlet of the inlet of the twisting path and the axial line of said second heater at the outlet contact end;  $l_2$  is the distance

between the point at which said yarn leaves the center of said fluid nozzle and the point at which the yarn is twist set multiplied by  $\cos \theta_2$ , and  $\theta_2$  is an angle formed by the line joining the point at which the yarn leaves said fluid nozzle with the point at which the yarn is twist set and the axial line of said fluid nozzle at the outlet center thereof.

14. The method of claim 13, wherein  $15^\circ \geq \theta > 0^\circ$ .

15. The method of claim 1, wherein the yarn is rotated by a fluid of the Reynolds number greater than 1,000 and up to 5,000 at the twisting portion of said fluid nozzle.

16. The method of claim 2, wherein a fluid of the Reynolds number greater than 1,000 and satisfying the following equation

$$(-0.0433 T_2 + 15.13)(2.02 \times 10^2) \times De^{0.200} \geq Re \\ \geq (0.040 T_1 - 0.045 T_2 + 4.2)(0.877 \times 10^2 De^{0.366})$$

wherein  $T_1$  is a first heat-setting temperature ( $^\circ C$ ),  $T_2$

5

10

15

20

is a second heat-setting temperature ( $^\circ C$ ), and  $De$  is the denier size of the yarn, is introduced into the twisting portion of said fluid nozzle.

17. The method of claim 16, wherein the Reynolds' number is maintained at a value greater than 1,000 and satisfying the following equation:

$$(-0.0450 T_2 + 14.90)(2.89 \times 10^2) De^{0.128} \geq Re \\ \geq (0.025 T_1 - 0.0450 T_2 + 8.40)(2.08 \times 10^2) De^{0.194}$$

18. The method of claim 1, wherein the thermoplastic synthetic filament yarn has a denier of 15 to 300.

19. The method of claim 1, wherein the filament yarn is a polyethylene-terephthalate yarn, poly-epsilon-caproamide yarn or a mixed yarn thereof.

20. The method of claim 1, wherein said fluid is air, nitrogen, carbon dioxide gas or mixtures thereof.

\* \* \* \* \*

25

30

35

40

45

50

55

60

65